

J. FEIGEN,  
BUILDING BOARD,  
APPLICATION FILED JAN. 16, 1915.

1,227,767.

Patented May 29, 1917.

Fig. 1.



Fig. 2.



Fig. 3.



WITNESSES:

A. H. Edgerton  
C. M. Merrick

INVENTOR

John Feigen.

BY

W. H. Farnsworth  
ATTORNEY

# UNITED STATES PATENT OFFICE.

JOHN FEIGEN, OF INDIANAPOLIS, INDIANA.

## BUILDING-BOARD.

1,227,767.

Specification of Letters Patent. Patented May 29, 1917.

Application filed January 16, 1915. Serial No. 2,671.

To all whom it may concern:

Be it known that I, JOHN FEIGEN, a citizen of the United States, and a resident of Indianapolis, county of Marion, and State of Indiana, have invented a certain new and useful Building-Board; and I do hereby declare that the following is a full, clear, and exact description thereof, reference being had to the accompanying drawings, in which like letters refer to like parts.

The object of this invention is to provide a veneer building board or block, to take the place of brick or stone in the construction of buildings, and which is so constructed as to have a hard or granite external surface, and yet the board or block is composed of material sufficiently yielding to enable it to be nailed into position against a board wall or frame and be held permanently in such position by the nails.

The chief feature of the invention consists in the body of the board being formed of cement mixed with mineral wool, and a layer of cement is adjacent said layer of mineral wool and cement combined, and adjacent said cement layer there is a layer of crushed granite, or the like, to form the external hard surface.

By using such boards, the construction of residences and other buildings can be greatly cheapened, as compared with those made of brick or stone, and yet a building formed of such boards will have the appearance of a stone building with an externally hard surface capable of resisting frost, temperature changes and other influences. Such boards can be very easily and readily nailed into place on a frame, and if any accident should happen to any one of said boards after the construction is finished, it can be readily removed and another board put in its place without affecting the remaining boards.

The nature of the invention will be understood from the accompanying drawings and the following description and claim.

In the drawings, Figure 1 is a section through a portion of such building board. Fig. 2 is a perspective view of a part of the wall showing the manner of erecting the same with said building boards. Fig. 3 is a vertical section through a portion of a wall and one building board secured thereto.

In detail, the building board consists of the main and inner layer 10, an outer or hard layer 11, and an intermediate or ce-

ment layer 12. The layer 10 is formed of cement, with mineral wool mixed therewith, so that said layer is always yielding. The layer 12 is relatively thin and is formed of cement, chiefly for the purpose of serving as a binder for the granite or hard layer 11.

The nature of the board will be understood from the following description of the process for making the same:

In the first place, the pallet of the mold is coated with a binder and crushed granite is sprinkled on said binder and then the pallet is turned upside down so that the particles of granite not bound by the binder fall away. Then smaller particles of crushed granite are sprinkled on the layers so far made and some of said particles adhere to the binder and the rest are allowed to fall away as before, and this process is continued until finally powdered granite is applied so as to fill up all spaces and make a substantially smooth and very thin granite layer. This is allowed to set for about two hours until it becomes hard.

In the next place, a liquid cement 12 is applied on said granite layer by a brush immediately before the mineral wool mixture is applied, and this layer 12 of cement gives strength and reasonable rigidity to the thin layer 11 of the granite.

Mineral wool is independently mixed with a relatively small amount of cement, sufficient to give the mineral wool reasonable stiffness and strength for handling and using it as a board, but so as to leave it compressible and yielding. Then, while the cement in layer 12 is fresh and unset, the combined mineral wool and cement is poured in a semi-liquid form into the mold, and the three layers are then allowed to set, and they become connected with each other and homogeneous.

The building board has the following peculiarities:

It is insulated against heat, because of the considerable quantity of mineral wool therein. It is tenacious and yielding, so that it can be nailed to the siding 13 of a house or frame structure, said siding being secured to uprights 14. The nails 15 readily go through the board when holes therefore are made in the hard external surface, and the heads thereof are obscured by rubbing a mixture of soft cement and granite over the same. Therefore, this building board is

put in place on the outside of a house somewhat like other kinds of building board, or secured on the inside of the house; but this makes the outer veneer of a wall of a permanent character. It does not break and a blow will cause a slight dent without breaking the external surface, as the material behind the external surface yields somewhat to the blow. If any particular board should be injured while erecting the wall, or afterward, it can be readily removed without displacing the other boards, and a new board put in place without difficulty. This is a peculiar advantage of this sort of building board. It is, furthermore, much cheaper than veneer bricks or stone, for which it is a substitute. With such granite-coated building boards, a wall of very attractive appearance from the outside will result, and it will resist temperature changes, rain, and the like, effectively.

While crushed granite is herein referred to, any crushed stone may be used, according to what is desired.

The invention claimed is:

A building board having its main portion consisting of mineral wool with a relatively small amount of cement therein so that said portion will maintain its shape and yet be resilient, a coating of cement on one surface of said mineral wool portion and adhering thereto, and crushed stone secured on said cement to form a hard external surface for said board, substantially as set forth.

In witness whereof I have hereunto affixed my signature in the presence of the witnesses herein named.

JOHN FEIGEN.

Witnesses:

J. H. WELLS,  
R. G. LOCKWOOD.